

# United States Patent [19]

Chang et al.

[11] 4,334,000

[45] Jun. 8, 1982

- [54] CYANINE AND DIANE DYE MIXTURE  
PROVIDES NEAR I. R. SENSITIVE, CHARGE  
TRANSPORT LAYER,  
ELECTROPHOTOGRAPHIC  
PHOTOCONDUCTIVE ELEMENT
- [75] Inventors: Mike S. H. Chang, Danbury; John T. Donoghue, Trumbull; Peter G. Edelman, Westport, all of Conn.
- [73] Assignee: Pitney Bowes Inc., Stamford, Conn.
- [21] Appl. No.: 218,389
- [22] Filed: Dec. 19, 1980
- [51] Int. Cl.<sup>3</sup> ..... G03G 5/14  
[52] U.S. Cl. ..... 430/58; 430/59;  
430/900
- [58] Field of Search ..... 430/58, 59, 900

[56]

## References Cited

### FOREIGN PATENT DOCUMENTS

2032637 5/1980 United Kingdom ..... 430/59

Primary Examiner—John D. Welsh

Attorney, Agent, or Firm—Melvin J. Scolnick; William D. Soltow, Jr.; Albert W. Scribner

[57]

## ABSTRACT

Dual layer organic photoconductive elements which are stable, have good negative charge acceptance and are sensitive over a broad range of the spectrum, including near the infrared band, and the process for preparing same. The charge-generating layer comprises a mixture of a charge-generating diane dye, such as Chlorodiane Blue, and a cyanine dye as a near-infrared sensitizer.

16 Claims, No Drawings

CYANINE AND DIANE DYE MIXTURE PROVIDES  
NEAR I. R. SENSITIVE, CHARGE TRANSPORT  
LAYER, ELECTROPHOTOGRAPHIC  
PHOTOCONDUCTIVE ELEMENT

BACKGROUND OF THE INVENTION

The present invention relates to the field of electro-photographic reproduction and, more particularly, to dual layer organic photoconductive elements such as belts, drums, webs, or the like, which are used in machines such as copying machines. Reference is made to U.S. Pat. Nos. 3,615,415, 3,824,099 and 4,150,987 for their discussion of the general field of the present invention and for their disclosures of some of the specific materials and procedures over which the present invention represents an improvement.

Aforementioned U.S. Pat. Nos. 3,824,099 and 4,150,987 relate to dual layer organic photoconductive elements comprising a conductive substrate such as a conductive paper, metallized plastic film or metal plate, supporting two basic layers, namely a charge-generating layer and a charge-transport layer. Either layer may be adjacent the conductive substrate, and an adhesive bonding layer may be interposed to bond the charge-generating layer.

During use, the photoconductive element is charged, exposed to light passed from the light reflective areas of an imaged original sheet to conduct away the charge in the exposed areas, and the charge-retaining or unexposed areas are either "inked" with electroscopic toner which is transferred to a copy sheet or are first transferred to a copy sheet and then "inked" with toner thereon. The toner is fused on the copy sheet to form fixed images corresponding to the images present on the original sheet.

Dual layer organic photoconductive elements were developed in order to provide extremely fast response to light exposure within the visible range of the spectrum. Preferred materials in this respect are diane blue dyes as the charge-generating organic chemicals of the charge-generating layer and p-type hydrazones or tri-aryl pyrazolines as the organic chemicals in the charge-transport layer.

Diane dyes have the general moiety structure as follows:



... wherein Z is a substituent group on the phenyl ring. Preferably, Z is selected from a group consisting essentially of hydrogen, alkyl, alkoxy and chlorine groups, more preferably hydrogen, methyl, methoxy and chlorine groups; and most preferably a chlorine group. Z is preferably attached to the ring in the 2 or 6 position.

The most preferred diane blue, Chlorodiane Blue, has chlorine as the Z group in the 2 position.

Chlorodiane Blue is a preferred charge-generating material because it has good stability and provides photoconductive elements having a relatively good shelf life or duration of storage prior to break-down and deterioration or loss of its charge-generating properties. Chlorodiane Blue also has superior light sensitivity and charge-generating properties over a broad portion of the visible light range, i.e., between about 400 m $\mu$  and 700 m $\mu$ . However, Chlorodiane Blue lacks adequate light sensitivity in the near-infrared range, i.e., between about 780 m $\mu$  and 1150 m $\mu$ .

Cyanine dyes are also known for use as charge-generating organic chemicals in dual layer organic photoconductive elements. Reference is made to the following Japanese Public Disclosure documents of the Japan KoKai Tokkyo Koho Company—Nos. 143,231/78; 21,343/79; 21,344/79; 21,345/79; 121,741/79 and 121,742/79. However, attempts to produce organic photoconductive elements according to these Public Disclosures, following the procedure outlined in Example 1 of U.S. Pat. No. 4,150,987 with the substitution of cyanine dye for Chlorodiane Blue, result in elements which do not have adequate negative charge acceptance with which therefore are substantially useless as photoconductive elements for duplication purposes. However, we discovered that by combining a certain amount of the cyanine dye with a diane dye, such as Chlorodiane Blue, charge-generating layers can be produced which have the desired negative charge acceptance and which are also sensitive over a broad range of the spectrum including near-infrared radiation.

SUMMARY OF THE INVENTION

The novel dual-layer organic photoconductive elements of the present invention were developed in order to provide improved sensitivity photoconductive elements having an extremely fast response to light exposure within a wide range of the spectrum including not only the visible spectrum but also extending into and including the near-infrared range, i.e., within a broad range of from about 400 m $\mu$  up to about 1150 m $\mu$ .

The present invention is based upon the discovery that while charge-generating layers containing Chlorodiane Blue are only highly sensitive to light exposure within the visible range, i.e., between 400 m $\mu$  and 700 m $\mu$  and thus are unsuitable for use with certain lasers as a light exposure source, and charge-generating layers based upon cyanine dye(s) lack the required negative charge acceptance of charge-generating layers based upon a diane dye such as Chlorodiane Blue, unexpectedly the combination of certain amounts of these charge-generating organic chemicals within the same charge-generating layer results in a layer which has the stability, negative charge acceptance and excellent sensitivity to light possessed by a diane dye, such as Chlorodiane Blue, but extending into and including a range of the near-infrared, i.e., within a range of between about 400 m $\mu$  and about 1150 m $\mu$ , and thus is suitable

for use with visible light sources as well as certain near-infrared light sources, such as certain lasers especially within a spectrum range of about 800 to about 850 m $\mu$ , as the light exposure source.

The novel combination of charge-generating organic chemicals comprises at least one diane dye and at least one cyanine dye. The basic moiety of the present cyanine dyes has a general structure as follows:



... wherein n is an integer selected from a range of 2 to 4 inclusive, preferably 3, Z is an anion, such as I<sup>-</sup> or ClO<sub>4</sub><sup>-</sup>; and A and B are non-fused or fused heterocyclic rings. Preferably A is selected from a group consisting essentially of:



-continued



... wherein R is an alkyl, substituted alkyl or aryl groups, preferably a methyl or ethyl group and X is selected from the group consisting of S, Se, O, NMe, NEt, CMe<sub>2</sub> and CEt<sub>2</sub>

Most preferably the cyanine dye is selected from the group consisting essentially of:



Generally, the effective weight percent of the cyanine dye sensitizer relative to the total weight of the charge-generating materials of the mixture can range between about 0.05% and 50.0%. Preferably, the diane dye is the major ingredient of the mixture and the cyanine dye comprises from about 1% to about 10% by weight of the mixture to produce the desired stability and high degree of sensitivity within a broad range of the spectrum including near infrared radiation.

The charge-generating layers of the present invention may be formulated and coated in any manner conventional in the art of dual layer organic photoconductive elements, such as taught for instances by U.S. Pat. Nos. 4,150,987 and 3,824,099. For example, the dye mixture may be dispersed and ground in a suitable volatile vehicle such as tetrahydrofuran, preferably at a concentration of between about 1% and 3%. The cyanine dye may be dissolved or dispersed in the vehicle.

A preferred embodiment involves the application of the charge-generating layer over an adhesive bonding layer present on a conductive support, which support may be a conventional aluminized polyethylene terephthalate film available from duPont under the registered trademark Mylar. A preferred adhesive bonding layer comprises a continuous coating of one or more adhesive resins known in the art, such as available from Goodyear under the registered trademark Vitel PE200 and PE307. Suitable conductive supports and bonding layers are disclosed in aforementioned U.S. Pat. No. 4,150,987. Alternatively, if desired, the present mixture of charge-generating dyes can be mixed with a desired adhesive resin in a proper ratio, followed by coating onto the conductive surface of the substrate. Optionally, the substrate can also have an adhesive layer precoated on its conductive surface before the dye layer coating, as discussed above.

As disclosed supra, the charge-transport layers suitable for use with the novel charge-generating layers of the present invention, and the method for preparing and applying the same in association with the present charge-generating layers, are conventional in the art and the pertinent disclosures of U.S. Pat. Nos. 3,615,415, 3,824,099 and 4,150,987 are incorporated herein by reference. The preferred charge-transport organic chemicals are the triaryl pyrazoline compounds of U.S. Pat. No. 3,824,099, such as 1-phenyl-3-[p-diethylaminostryl]-5-[p-diethylamino phenyl]-pyrazoline, and the hydrazone compounds of U.S. Pat. No. 4,150,987, such as p-diethylaminobenzaldehyde-(diphenyl hydrazone). The charge-transfer chemical is dispersed or dissolved in a solution of one or more resinous binder materials and the charge-transport layer is applied and dried by evaporation of the volatile solvent, in known manner.

The following example is given to illustrate the present invention but is not to be considered as a limitation of the scope of the invention.

#### EXAMPLE 1

The general procedure disclosed in Example 1 of U.S. Pat. No. 4,150,987 was followed to prepare an organic photoconductive element according to the present invention except that the charge-generating layer was formulated and coated in the following manner.

The charge-generating coating composition was produced by mixing together 5.0 mg. of a cyanine dye, commercially-available from Eastman Organic Chemicals under the designation IR-140, and 0.267 g. of Chlorodiane Blue and adding to the mixture 15 ml. of tetrahydrofuran as a volatile vehicle to form a dispersion. The dispersion was ball milled for eight hours in a 2-ounce

jar using  $\frac{1}{8}$ " chrome-plated balls until the maximum particle size of the dye particles is 0.25 mil or less, as measured with a fineness of Grind Measurer of the Precision Gauge and Tool Co.

The conductive substrate of aluminized Mylar is first coated with an adhesive bonding layer comprising a mixture of equal parts by weight of Vitel PE-200 and Vitel PE-307, the bonding layer having a weight of about 13 mg/ft<sup>2</sup> over the aluminized surface of the Mylar substrate.

The ground dye mixture dispersion is applied over the adhesive bonding layer using a Gardner-Ultra Applicator draw down blade with the blade set at a gap of 10, i.e., 1 mil. the dye coating was dried by evaporation of the vehicle to form the charge-generating layer.

Thereafter, a hydrazone charge-transfer layer was formulated and applied over the dye layer in the manner disclosed in Example 1 of U.S. Pat. No. 4,150,987 in a coat weight of about 1.8 g/ft<sup>2</sup>.

The organic photoconductive element of Example 1 supra was compared with the photoconductive element product in exact accordance with Example 1 of U.S. Pat. No. 4,150,987 with respect to photosensitivity to light in the near-infrared region of the spectrum using a Victoreen Electrostatic Paper Analyzer with a Kodak #87 filter positioned between the tungsten lamp and the sample.

The amount of energy required to discharge the charge acceptance from -400 volts to -200 volts, i.e., 35 E  $\frac{1}{2}$ , was measured in identical fashion for each of the samples. The amount of energy required by the sample produced according to Example 1 herein was determined to be about 950  $\mu$ J/cm<sup>2</sup>, whereas the amount of energy required by the sample produced according to Example 1 of U.S. Pat. No. 4,150,987 was determined to be about 7100  $\mu$ J/cm<sup>2</sup>, i.e., nearly 7.5 times less sensitivity to the near-infrared radiation transmitted by the Kodak #87 filter.

Variations and modifications of the present invention will be apparent to those skilled in the art within the scope of the present claims.

We claim:

50 1. A photoconductive element which is extremely sensitive to exposure to light rays in the near-infrared region of the spectrum, said element comprising an electroconductive support, a charge generating layer comprising a mixture of at least one cyanine dye and at least one diane dye in which the weight percent of cyanine dye relating to the total weight of said dye mixture ranges between about 0.05% and 50.0%, said cyanine dye having a general structure of the basic moiety as follows:



65 . . . wherein n is an integer selected from a range of 2 to 4 inclusive, Z<sup>-</sup> is an anion, and A and B are non-fused or fused hetero-cyclic rings, wherein A is selected from the group consisting of:



... and B= is selected from the group consisting of:



4. A photoconductive element according to claim 1, 2 or 3 in which said diane dye comprises Chlorodiane Blue.

5. A photoconductive element according to claim 1 in which said weight percent of cyanine dye ranges between about 1% and 5% of said dye mixture.

-continued



... wherein R is selected from the group alkyl, substituted alkyl and aryl groups and X is selected from the group S, Se, O, NMe, NEt, CMe<sub>2</sub> and CEt<sub>2</sub>, and a charge transport layer comprising a conventional organic chemical capable of transporting electrical charges generated by said charge generating layer in areas of said element exposed to said light rays.

2. A photoconductive element according to claim 1 in which said n is 3.

3. A photoconductive element according to claim 1 in which the cyanine dye is selected from the group consisting of:

6. A photoconductive element according to claim 1 in which said electroconductive support comprises a metalized plastic film.

7. A photoconductive element according to claim 1 or 6 in which said electroconductive support carries an adhesive resinous layer which bonds said charge-generating layer to said electroconductive support.

8. A photoconductive element according to claim 1 in which said organic chemical of the charge-transport layer is selected from the group consisting of triaryl pyrazolines and hydrazones.

9. Process for producing a photoconductive element which is extremely sensitive to light rays in the near-infrared region of the spectrum, said element comprising an electroconductive support, a charge generating layer and a charge transport layer comprising a conventional organic chemical capable of transporting electrical charges generated by said charge generating layer in areas of said element exposed to said light rays, comprising the step of producing said charge generating layer by mixing together a cyanine dye and a diane dye in a coating composition in which the weight percent of cyanine dye relative to the total weight of said dye mixture ranges between about 0.05% and 50.0%, said cyanine dye having a general structure of the basic moiety as follows:



... wherein n is an integer selected from a range of 2 to 4 inclusive, Z<sup>-</sup> is an anion, and A and B are non-fused or fused hetero-cyclic rings, wherein A is selected from the group consisting of:



-continued



... and B is selected from the group consisting of:



45 ... wherein R is selected from the group alkyl, substituted alkyl and aryl groups and X is selected from the group S, Se, O, NMe, NEt, CMe<sub>2</sub> and CEt<sub>2</sub>, and applying said composition as a uniform thin layer.

50 10. Process according to claim 9 in which said n is 3.

11. Process according to claim 9 in which the cyanine dye is selected from the group consisting of:

-continued



which is evaporated to form said charge-generating layer.

20 15. Process according to claim 14 in which said dye mixture and volatile vehicle are ground to form a coating composition comprising a dispersion of dye particles having a maximum particle size of about 0.25 mil.

16. Process according to claim 9 which comprises coating said electroconductive support with a continuous bonding layer of adhesive resin and applying said charge-generating layer to the surface of said bonding layer.

\* \* \* \* \*

30

35

40

45

50

55

60

65